

1

3,036,003

### LUBRICATING OIL COMPOSITION

Joseph Arthur Verdol, Dolton, Ill., assignor, by mesne assignments, to Sinclair Research, Inc., New York, N.Y., a corporation of Delaware  
No Drawing. Filed Aug. 7, 1957, Ser. No. 676,719  
7 Claims. (Cl. 252—33.4)

This invention relates to the improvement of mineral oil compositions, and more particularly to the improvement of lubricating oils containing basic salts of oil-soluble sulfonates by the addition thereto of an effective inhibitor-detergent type additive agent.

A variety of additive agents have been designed for the addition to lubricating oils whereby one or more properties of the oil would be improved. For example, metallic detergents in lubricating oils adapted for use in internal combustion engines have been found to improve the vehicle operation by preventing or retarding corrosion, piston ring sticking, cylinder wear, and carbon and varnish formation. Among the detergent-dispersant type additives used for this purpose are the so-called basic salts or soaps of oil-soluble petroleum sulfonic acids. These basic compounds are well-known materials and are prepared by neutralizing the acid with an excess of neutralizing agent which is in the form of the oxide, hydroxide or carbonate of the desired metal, so as to obtain a product which contains an amount of metal in excess of that theoretically required to replace the acidic hydrogens of the acid. Such detergents have been used with much success in lubricating oils for internal combustion engines. However, in lubricating oils containing other additive agents, for example, anti-oxidants such as alkyl phenol sulfides and their metal salts, these basic detergent materials often have the objectionable feature of being fairly corrosive toward metals and alloys which are widely used as bearing metals.

In accordance with this invention I have found that if a condensation product of an alkylene polyamine, an aldehyde and substituted phenol, or an alkaline earth metal salt thereof, is added to a mineral lubricating oil which contains a basic alkaline earth metal salt of an oil-soluble petroleum sulfonate, the combination of additives will effectively reduce the tendency of such oils to undergo oxidation, formation of gums, sludges, and other deterioration which occurs when the oil is used in internal combustion engines. When the alkaline earth metal salts of the condensation product are used in conjunction with the oil-soluble sulfonates good performance is obtained with respect to engine cleanliness and bearing corrosion. The metallic derivatives have been found especially suited as detergent-inhibitors and can be used in amounts appreciably less than other additives known in the prior art in order to obtain a desired level of performance. As ashless detergent-inhibitors, the non-metallic condensation products do not have the objectionable feature of leaving a deposit or ash in internal combustion engines and are highly desirable for inhibiting oxidation.

In order to obtain the oil-compatible, i.e. soluble, dispersible or miscible without continuing agitation, condensation products used in accordance with this invention, an alkylene polyamine, formaldehyde and substituted phenol are reacted together at an elevated tempera-

2

ture, such as a temperature in the range of 100 to 350° F., in the presence or absence of a solvent. The reactants are employed in a ratio of at least about 0.5 mole of each of phenol and aldehyde for every basic nitrogen atom present in the alkylene polyamine, with the upper limit being about 2 moles of phenol and aldehyde for each nitrogen atom in the amine. The condensation products are essentially linear and thus are not condensed to an infusible and insoluble stage such as occurs in the usual phenol-formaldehyde condensation reactions, but have reactive phenolic hydroxy groups which remain unsubstituted or which have hydroxyl hydrogens replaced with an alkaline earth metal. It is believed that the molecular weight of the product is in the range of 500 to 5000. The desired metal of the alkaline earth group is preferably introduced by reaction of its oxide or hydroxide with the condensation product.

As indicated above, the reactants are maintained in a ratio of at least about 0.5 mole of phenol and aldehyde for every basic nitrogen atom present in the amine. In this manner the products thus obtained have been found to exhibit good oil solubility, wide molecular weight distribution and varying amounts of nitrogen. As an example, the condensation of 3 moles of p-t-octylphenol and formaldehyde with one mole of diethylenetriamine affords a product which may be illustrated as:



in which R is the alkyl group of the phenol. However, when the reaction is carried out using a ratio of 2 moles of the same aldehyde and phenol per mole of amine, a product of lower molecular weight and higher nitrogen content is formed, which is represented as:



or



55

in which R is the alkyl group of the phenol. Similarly, when tetraethylenepentamine is used as the alkylene polyamine source in the above condensation reaction, a series of high molecular weight condensation products are obtained. Thus, a condensation product formed from the reaction of 4 moles of octylphenol and formaldehyde per mole of tetraethylenepentamine affords a product comprised of several compounds the major portion of which are shown below:





Since the ratio of reactants employed in the above condensation were such that one secondary nitrogen atom would remain unsubstituted, a mixture of products could not be precluded and it is believed that the above formulations predominate although positioned isomers other than those shown are also possible. Similarly, when the same reaction is carried out using a higher ratio of reactants, a condensation product higher in molecular weight and lower in nitrogen content is obtained. Thus, the condensation product obtained by reacting 5 moles of octylphenol and formaldehyde with one mole of tetraethylenepentamine is illustrated by the probable structure shown below:



The condensation reaction of my invention takes place at temperatures of about 100 to 350° F., preferably at temperatures of about 100 to 270° F., and can be conveniently carried out in the presence of any suitable solvent such as benzene or toluene which can be recovered from the reaction product. If desired, the reaction may be carried out in a mineral oil whereby the condensation product is recovered as a mineral oil concentrate. No special equipment is required for the reaction and any suitable pot type reactor can be employed.

As previously stated, the condensation products of my invention are characterized as either having reactive phenolic hydroxy groups which remain unsubstituted or which have their hydroxyl hydrogen replaced with an alkaline earth metal compound. The oil-soluble calcium salts are particularly effective for imparting thermal and oxidative stability to mineral oils and can be prepared by neutralization of the condensation product with a basic compound of calcium, such as calcium hydroxide, or by neutralization with a metal oxide or hydroxide followed by preparation of the calcium salt by methathesis. Preferably when carrying out the neutralization of the condensation product additional mineral oil of the type employed in preparing a mineral oil concentrate is added to the reaction mixture together with lime and a small amount of water to facilitate the neutralization.

The alkylene polyamines employed in the preparation of the condensation product are represented by the general formula:



in which R is a divalent alkyl radical, substituted or unsubstituted, containing about 2 to 6 carbon atoms, and n is an integer from 1 to 10. Typical amines of the above type include diethylenetriamine, triethylenetetramine, tetraethylenepentamine, etc. Other suitable amines are the polymerized ethylene imines having a molecular weight of from about 1000 to 40,000.

The substituted phenols contemplated herein are the

alkylated monohydric phenols having at least one alkyl group of sufficient length to impart oil-solubility to the condensation products. Such phenols are further characterized as having at least one ortho or para position which is available as a reaction site in the nucleus. The alkylated phenols can be prepared by well-known methods as, for example, by alkylating phenol or the homologs thereof with an alkyl halide in the presence of a Friedel-Crafts catalyst. Representative alkyl phenols which can be employed are those in which the alkyl group contains from 4 to 20 carbon atoms, and preferably those having 8 to 20 carbon atoms such as, for example, n-amyl phenol, diethyl phenol, octyl phenol, nonyl phenol, p-tert-octyl phenol, a

mixture of phenols, and the like. If desired, the alkylated phenols may also contain one or more substituent groups such as nitro, alkoxy, and the like.

As previously mentioned the inhibitor detergent agents of this invention are employed in lubricating oil compositions which contain basic salts or soaps of oil-soluble sulfonic acids. The basic salts or soaps which are employed are preferably the alkaline earth metal salts of petroleum sulfonic acids, and more particularly the calcium and barium salts. The oil-soluble sulfonic acids, referred to as mahogany acids, are well known and may be obtained by sulfonating a suitable petroleum distillate with oleum or sulfur trioxide to obtain a 10 to 20 percent concentrate of mahogany acids in the acid oil. The useful mahogany acids generally have a molecular weight of from about 300 to 500, or more, and may be converted into the basic salts by neutralization of the acid oil with an excess of basic barium or calcium compound to obtain basic sulfonates having a higher metal content than the normal salt. Generally, the barium neutralizing agent is reacted with the mahogany acids in a proportion of at least about 1.5 times the theoretical amount required to obtain the normal salt while with calcium the proportion is at least about 1.1. The amount of basic alkaline earth metal sulfonate used in the mineral oil base depends upon the nature of the base stock employed and its service application. Generally, the basic metal sulfonate is used in a range of from about 0.5 percent to 10 percent by weight on a dry soap basis. In the lubricating compositions of this invention the basic sulfonate is added in a sufficient amount to effect a metal content of about 0.2 percent to 2.0 percent by weight.

The preferred inhibitor-detergent additive agents of this invention are those reaction products obtained by condensing a mixture of tetraethylenepentamine, octyl phenol and formaldehyde in a ratio of at least 4 moles, and preferably 5 moles, of phenol and aldehyde to 1 mole of amine at a temperature of about 100 to 270° F. Although the additive agents can be prepared as a separate product,

## 5

for example, in solvents such as benzene or toluene, it is preferred to produce the additive by reaction in a solvent refined neutral oil so as to obtain a mineral oil concentrate. The resulting concentrate, either alone or as the alkaline earth metal salt, preferably the calcium salt, may be incorporated in the desired lubricating oil in a small proportion sufficient to impart the desired function of the additive. As detergent-inhibitors, alone or in combination with other additives, the metal salts are usually blended with the oil in an amount to provide a calcium level of about 0.01 to 0.5 percent by weight. As ashless detergents which can be used as such or in combination with other well-known detergents, and which further exhibit oxidation inhibiting properties as well as good dispersant properties, the condensation products are usually blended in an amount of about 0.1 to 5.0 percent by weight based on the weight of mineral oil.

The following examples serve to illustrate more clearly the preparation of the condensation products of my invention and the desirable results obtained by their use in mineral oils.

## Example I

412.6 grams (2 moles) of p-tert-octylphenol, 94.7 grams (0.5 mole) of tetraethylenepentamine and 750 grams of a solvent-treated Mid-Continent neutral oil were placed in a 3-liter, 4-necked flask equipped with a heater, thermometer and Dean Stark trap. The mixture was heated to about 185° F. and two moles of formalin were added over a period of one hour. The temperature was maintained at 200 to 230 F. for an additional hour and dehydration of the reaction mixture was then effected at 240-260° F. under a slight vacuum. The total reaction time was three hours. The product, identified as 58a, was an extremely viscous liquid which was obtained as a 40 percent concentrate in a yield of 98.5 percent of the theoretical. Analysis showed the following properties:

Percent nitrogen ----- 2.56  
Acid No. pH 11 ----- 0.05  
Base No. pH 4 ----- 60.3

Forty grams of 58a was blended in 360 grams of a Mid-Continent neutral oil and tested for viscosity and pour point characteristics. The following data were obtained:

KV centistokes:  
100° F. ----- 43.8  
210° F. ----- 6.21  
Pour point ----- °F. 5  
VI ----- 96

Two hundred and twenty-eight grams of product 58a (40 percent concentrate) and 1 mole of calcium hydroxide containing 80 grams of water were placed in an apparatus similar to that described above. The mixture was heated with stirring to about 300° F. and an additional 322 grams of the Mid-Continent solvent refined neutral oil was added. Heating was continued at 300° F. for about 3 hours until dehydration was complete. One percent by weight of Super-Cel was added to the mixture with stirring and the mixture was filtered hot in vacuo through a heated Buchner funnel. The resulting product (as an 18 percent concentrate) was a clear, amber colored liquid, having the following analysis:

Percent calcium (found) ----- 0.84  
Initial pH ----- 10.6  
Acid No. pH 11 ----- 0.00  
Base No. pH 4 ----- 46.5  
KV:  
100° F. ----- cs. 209.3  
210° F. ----- 14.09  
Pour point ----- °F. 70

## Example II

In a 5-liter, 4-necked flask, equipped as described in Example I was placed 825.2 grams (4 moles) of p-tert-octylphenol, 1359 grams of a Mid-Continent solvent re-

## 6

fined neutral oil and 189 grams (1 mole) of tetraethylenepentamine. The mixing of the above ingredients caused a slight rise in temperature of the reaction mixture. The mixture was heated to about 165° F. and 4 moles of formalin (37 percent) were added over a period of about two hours. The mixture was then heated for three hours while continuously increasing the temperature. At the end of the three-hour period, a maximum temperature of about 345° F. was achieved and dehydration was complete. The product, identified as 58aa and prepared as a 44 percent concentrate, was a viscous, light amber colored liquid, and weighed 2080 grams (98 percent yield). Analysis showed the following properties:

Percent nitrogen (found) ----- 2.79  
Acid No. pH 11 ----- 0.4  
Base No. pH 4 ----- 71.0

To a mixture of the above product 58aa (1025 grams) and 1000 grams of a Mid-Continent solvent refined neutral oil was added, with stirring, 2 moles of calcium hydroxide and 100 grams of water. The reaction mixture was heated at 230 to 250° F. for two hours, and the temperature was then raised until a maximum temperature of about 330° F. was attained at complete dehydration. The product was filtered hot, in vacuo, employing Super-Cel. The product was a clear amber liquid and was a 22.5 percent concentrate of the calcium salt of product 58aa. Analysis showed the following:

Percent calcium (found) ----- 1.30  
Acid No. pH 11 ----- 0.00  
Base No. pH 4 ----- 73.6  
Initial pH ----- 11.2

## Example III

In a 5-liter, 3-necked flask, equipped with a heater, stirrer, thermometer and dropping funnel, was placed 1237.8 grams (6 moles) of p-tert-octylphenol and 206.32 grams (2 moles) of diethylenetriamine. The amine was added slowly over a period of 30 minutes to the octylphenol which was heated to about 175° F. The temperature was about 185° F. after the amine addition was completed, and the addition of the formalin (6 moles, 37 percent) was initiated. The formalin was added over a period of one hour and the reaction mixture was heated slowly to about 320° F. until dehydration of the mixture was completed. The hot reaction product, identified as 58c and obtained as 100 percent concentrate, was poured from the reaction flask into a stainless steel beaker where it solidified to an amber colored material. Analysis of the product showed the following properties:

Acid No. pH 11 ----- 1.40  
Base No. pH 4 ----- 132.3  
Percent nitrogen (found) ----- 5.38  
Initial pH ----- 9.0

The above product 58c was dissolved in a Mid-Continent solvent refined neutral oil and neutralized with calcium hydroxide in the usual manner to give a 34 percent concentration of product 58c. The filtered calcium salt showed the following properties:

Acid No. pH 11 ----- 0.0  
Base No. pH 4 ----- 101.8  
Initial pH ----- 11.5  
Percent nitrogen (found) ----- 1.71

KV:  
100° F. ----- cs. 1023.8  
210° F. ----- cs. 28.2  
Pour point ----- °F. 5  
Percent calcium (found) ----- 2.0

## Example IV

By employing the technique described above for the preparation of product 58c, only using a ratio of 2 moles of aldehyde and phenol per mole of amine, a product of low molecular weight and high nitrogen content is

formed. Thus, when 6 moles of p-tert-octylphenol (1236 grams) were condensed with 309.48 grams (3 moles) of diethylenetriamine and 6 moles of formalin, a light amber-colored product, identified as 58d, was obtained which had the following analysis:

|                  |       |
|------------------|-------|
| Percent nitrogen | 7.62  |
| Acid No. pH 11   | 0.35  |
| Base No. pH 4    | 207.6 |
| Initial pH       | 10.0  |

582 grams of product 58d were blended in 882 grams of a Mid-Continent solvent refined neutral oil and heated to 167° F. 5 moles of calcium hydroxide and 100 grams of water were added to the mixture. The mixture was then heated for three hours while slowly increasing the temperature until dehydration was complete at a temperature of about 306° F. The calcium salt of product 58d was obtained as a 41.5 percent concentrate in the Mid-Continent oil and had the following characteristics:

|                  |       |
|------------------|-------|
| Percent calcium  | 2.86  |
| Percent nitrogen | 2.75  |
| Acid No. pH 11   | 0.00  |
| Base No. pH 4    | 154.7 |
| Initial pH       | 11.9  |

KV:

|         |         |
|---------|---------|
| 100° F. | 3,767.7 |
| 210° F. | 64.9    |

Pour point ° F. 10

147 grams of formalin (37 percent) was added dropwise over a period of 15 minutes. The reaction mixture was then heated to about 200 to 300° F. until dehydration was complete. The reaction product was a clear, straw colored, viscous liquid, which was converted to the calcium salt by adding 3 moles of calcium hydroxide, 110 ml. of water, and 200 grams of a Mid-Continent solvent refined neutral oil. The mixture was heated over a period of three hours from 190 to 300° F. at which temperature dehydration was complete. Analysis of the condensation product showed the following:

|                  |      |
|------------------|------|
| Percent calcium  | 1.15 |
| Percent nitrogen | 1.37 |
| Acid No. pH 11   | 1.76 |
| Base No. pH 4    | 55.5 |
| Initial pH       | 10.0 |

The benefits derived from the condensation products prepared in accordance with this invention are illustrated in the following tables by the tabulated results obtained from the Railroad Oxidation Test as applied to the calcium salts of the additive agents as prepared in Examples I, II and III. This test is of low temperature and long duration and consists of passing 5 liters of oxygen per hour into 300 ml. of oil blend of 285° for 144 hours. Fifty milliliters of makeup oil is added at 48 hours and 96 hours. The test is carried out in the presence of a 1" x 3" steel back copper lead catalyst.

TABLE I

| Sample number                                            | 8140            | 10232                 | 8143           | 8196            | 8197            | 8199           | 8200            |
|----------------------------------------------------------|-----------------|-----------------------|----------------|-----------------|-----------------|----------------|-----------------|
| Base oil:                                                |                 |                       |                |                 |                 |                |                 |
| Percent Coastal <sup>1</sup>                             | 50              | 50                    | 50             | 50              | 50              | 50             | 50              |
| Percent Mid-Continent <sup>2</sup>                       | 50              | 50                    | 50             | 50              | 50              | 50             | 50              |
| Additives:                                               |                 |                       |                |                 |                 |                |                 |
| Percent basic calcium sulfonate <sup>3</sup>             | 12 (0.07% Ca).  | 12 (0.07% Ca).        | 12 (0.07% Ca). | 12 (0.07% Ca).  | 12 (0.07% Ca).  | 12 (0.07% Ca). | 12 (0.07% Ca).  |
| Percent Oronite 216 <sup>4</sup>                         | 2.3 (0.10% Ca). |                       |                |                 |                 |                |                 |
| Percent calcium phenol sulfide (laboratory preparation). |                 | 3.6 (0.1% Ca).        |                |                 |                 |                |                 |
| Percent calcium salt of 58a, Example I.                  |                 |                       | 8.3 (0.1% Ca). |                 |                 |                |                 |
| Percent calcium salt of 58c, Example III.                |                 |                       |                | 5.0 (0.10% Ca). | 2.5 (0.05% Ca). |                |                 |
| Percent calcium salt of 58aa, Example II.                |                 |                       |                |                 |                 |                | 7.7 (0.15% Ca). |
| Railroad oxidation used oil tests:                       |                 |                       |                |                 |                 |                |                 |
| Vis./100° F.                                             | 2,200           | 8,413                 | 984            | 1,018           | 1,016           |                | 1,051           |
| Vis./inc. percent                                        | 170             | 57.2                  | 2.07           | 6.5             | 4.7             |                | 10.5            |
| Acid number D-974                                        | 14.18           | 7.81                  | 0.94           | 0.92            | 0.92            |                | 1.67            |
| Initial pH                                               | 3.1             |                       | 8.1            | 7.1             | 6.8             |                | 6.2             |
| Pentane insol., percent                                  | 5.724           | 0.423                 | 0.012          | 0.066           | 0.010           |                | 1.719           |
| Weight change cat., mg                                   | -635            | -2,416                | 2.6            | -72             | -22.2           |                | -112.5          |
| Tube varnish or sludge                                   |                 | Some sludge and varn. |                | No sludge       |                 |                | Clean           |
| Catalyst appearance                                      | No sludge       |                       | No sludge      | do              |                 |                | No sludge       |

<sup>1</sup> An acid-treated Coastal Oil Blend having a viscosity of about 90 SUS at 210° F.

<sup>2</sup> A solvent-refined oil blend having a viscosity of about 90 SUS at 210° F.

<sup>3</sup> Employed as a 12% concentrate and blended to a calcium level of .07% by weight.

<sup>4</sup> Calcium phenol sulfide.

To illustrate the versatility of the condensation reaction of alkylpolyamines with substituted phenols and formaldehyde, a condensation reaction was carried out employing polymerized ethylene imine as the amine source in the reaction. The polymerized ethylene imine was obtained from Hansborg and Company and was furnished as a 50 percent aqueous solution, having a molecular weight distribution of 30,000 to 40,000. The procedure given below was employed for the preparation of the calcium salt of the condensation product of nonylphenol with polymerized ethylene imine and formaldehyde.

#### Example V

Into a 3-liter, 4-necked flask equipped with a heater, stirrer, Dean Stark trap and dropping funnel was placed 390 grams of nonylphenol and 95 grams of polymerized ethylene imine. Six hundred grams of a Mid-Continent solvent refined neutral oil was added to the mixture and

60 The data in Table I above show that the incorporation of calcium additives 58a, 58aa and 58c in the oil blends imparted excellent thermal and oxidation stability to blends containing a basic calcium sulfonate detergent. In every case where a calcium additive of this invention was used in an oil blend, a satisfactory railroad oxidation test was obtained. In contradistinction to this behavior, experimental oils formulated with conventional inhibitors such as a calcium phenol sulfide or Oronite 216 (a sulfurized calcium phenate) gave unsatisfactory Railroad Oxidation Tests. The latter blends gave tests characterized especially by high viscosity increases and high acid numbers. A major point of importance was demonstrated by test blend 8197, in which the calcium salt of product 58c was used at a concentration of 0.05 percent calcium. This test blend performed extremely well al-

though it contained one-half of the normal amount of calcium. Thus, in combination with a basic sulfonate, the calcium additives can be utilized in much lower concentrations than with conventional inhibitors and yet provide superior performance as oxidation inhibitors. Moreover, as shown hereinafter, additional tests which have been carried out with the non-metallic condensation products have shown that in combination with typical pro-oxidants, extremely good results have been obtained in the Railroad Oxidation Tests.

The following data presented in Table II show the results obtained in Railroad Oxidation Tests carried out on blends containing a detergent (basic calcium sulfonate) and a supplementary inhibitor together with the calcium additive 58a as prepared in Example I. Similar blends formulated with several different calcium phenol sulfides instead of the calcium salt of product 58a were also tested for comparison.

As shown below, the data obtained again illustrate the superior performance of the additive agent 58a over the two commercial additives above described, even in the presence of a supplementary inhibitor. The addition of a supplementary inhibitor to the blends formulated with calcium 58a and basic calcium sulfonate imparted no additional stability to the oil blends (compare Tables I and II). Thus another outstanding feature of the novel calcium additives is their ability to impart cleanliness and stability to lubricating oils without the addition of supplementary inhibitors.

Varnish and sludge rating----- 97.5.  
Bearing loss avg. mg./whole bearing----- 22.2.  
Color and condition of bearing----- Copper colored-clean.

## USED OIL TESTS

|   |                |      |
|---|----------------|------|
| 5 | Acid number    | 2.66 |
|   | Pentane insol. | .424 |
|   | Benzene insol. | .290 |
|   | Insol. resin   | .134 |

Vis. increase at 100° F. percent 17.4

<sup>1</sup> Coastal—Acid treated coastal oil blends of oils approximately 61 and 75 SUS vis./210° F., respectively.

<sup>2</sup> Mid-Continent—A blend of Mid-Continent solvent treated neutral oil and bright stock of 100 SUS vis./210° F.

<sup>3</sup> As prepared in Example I.

As shown in Table III the new detergent-inhibitor additives impart excellent stability and oxidation resistance as indicated by a total varnish and sludge rating of 97.5. As further shown in the data under bearing loss in these tests, which indicates the amount of bearing corrosion expressed in milligrams loss in weight of a standard bearing, the novel additives effectively suppress degradation of the lubricating oil composition and corrosion of bearing metals resulting from oxidation in the presence of the bearing metals under severe service conditions.

Additional tests were carried out to determine the ability of the novel additives to act as dispersants by maintaining insolubles, etc. in a state of suspension. The additives prepared in Example I, including condensation product 58a and the calcium salt thereof, both were compared with a basic barium petroleum sulfonate and a commercial detergent designated as compound x. The data were obtained by employing the Carbon Black Suspension Test, the procedure for which is as follows:

TABLE II

| Sample number                                           | 10240           | 10154          | 10135          | 8144          | 8145          | 10285 | 10134          |
|---------------------------------------------------------|-----------------|----------------|----------------|---------------|---------------|-------|----------------|
| Base oil:                                               |                 |                |                |               |               |       |                |
| Percent Coastal <sup>1</sup>                            | 50.             | 50.            | 50.            | 50.           | 50.           | 50.   | 50.            |
| Percent Mid-Continent <sup>2</sup>                      | 50.             | 50.            | 50.            | 50.           | 50.           | 50.   | 50.            |
| Additives:                                              |                 |                |                |               |               |       |                |
| Percent Oronite 216 <sup>3</sup>                        | 2.45 (.10% Ca.) | 2.3 (.10% Ca.) |                |               |               |       |                |
| Percent calcium phenol sulfide <sup>4</sup>             |                 |                | 3.27 (.1% Ca.) |               |               |       | 3.27 (.1% Ca.) |
| Percent calcium phenol sulfide (laboratory preparation) |                 |                |                |               |               |       |                |
| Percent calcium salt of 58a, Example I                  |                 |                |                | 8.3 (.1% Ca.) | 8.3 (.1% Ca.) |       |                |
| Percent basic calcium sulfonate <sup>5</sup>            | 12.             | 12.            | 12.            | 12.           | 12.           | 12.   | 12.            |
| Percent inhibitor <sup>6</sup>                          | 1.75            | 2.5            | 2.5            | 1.75          | 2.5           | 1.75  | 1.75           |
| Railroad oxidation used oil tests:                      |                 |                |                |               |               |       |                |
| Vis./100° F.                                            | 826.1           | 1,060          | 1,101          | 1,012         | 1,071         | 842.7 | 1,106          |
| Vis./inc., percent                                      | 43.2            | 67             | 49.7           | 5.0           | 11            | 35.6  | 55.4           |
| Acid number D-974                                       | 5.63            | 6.16           | 7.66           | 2.09          | 4             | 6.51  | 7.09           |
| Initial pH                                              |                 | 1.4            | 1.3            | 6.2           | 3.5           |       | 1.3            |
| Pentane insol., percent                                 | 2.707           | 2.517          | 4.2            | 0.00          | 0.227         | 3.38  | 3.62           |
| Cat. weight change, mg.                                 | -13.3           | -6.1           | -9.1           | -43           | -145          | 11.7  | -13.1          |
| Tube varnish or sludge                                  |                 |                |                | No sludge     | Slight sludge |       |                |
| Catalyst appearance                                     |                 |                |                | do            | No sludge     |       |                |

<sup>1</sup> See Table I.

<sup>2</sup> See Table I.

<sup>3</sup> See Table I.

<sup>4</sup> A commercial calcium phenol sulfide having an hydroxyl value of 130.7 and a sulfur analysis of 6.1%. As employed herein, this material is neutralized with calcium hydroxide to obtain a product having 3.06% calcium, 5.62% sulfur and a Base No. pH 4 of 77.8.

<sup>5</sup> See Table I.

<sup>6</sup> A commercial inhibitor (Pinene-P<sub>2</sub>S<sub>6</sub>-phenol-SCl<sub>4</sub>-alcohol-reaction product, neutralized with lime).

TABLE III  
Chevrolet L-4 Engine Test Results Run at 280° F.  
Crankcase Sump

## FRESH OIL COMPOSITION

|                                                                  |                   |     |
|------------------------------------------------------------------|-------------------|-----|
| 750 Coastal <sup>1</sup>                                         | percent by volume | 18  |
| 1200 Coastal <sup>1</sup>                                        | do                | 42  |
| 100 Mid-Continent <sup>2</sup>                                   | do                | 40  |
| 6.6% calcium 58a; 12% basic calcium sulfonate conc. <sup>3</sup> | percent Ca        | 0.1 |

| VARNISH RATING | SLUDGE RATING |
|----------------|---------------|
| Piston skirt   | 9.5           |
| Rocker cover   | 10.0          |
| Push rod cover | 10.0          |
| Cylinder wall  | 10.0          |
| Crankcase      | 10.0          |

Total 49.5 Total 48.0

A given weight of the additive was blended in a mixture comprising 25 ml. of a Mid-Continent refined neutral oil and 25 ml. of kerosene. To this mixture was then added 0.25 gram of carbon black. The mixture was homogenized three times through a hand homogenizer and heated with stirring for five minutes at a temperature of about 300° F. It was then poured into a 50 ml. graduated cylinder and permitted to stand in an oven at about 150° F. for 17 hours. After this time, the level of carbon black in the cylinder was observed. Table IV below shows the results of these tests.

TABLE IV  
Carbon Black Suspension Tests

| Composition of Blend                                                                                   | Level of carbon black after 17 hrs. at 150° F., ml. |
|--------------------------------------------------------------------------------------------------------|-----------------------------------------------------|
| 1. Kerosene plus Mid-Continent solvent refined oil blend having a viscosity of about 90 SUS at 210° F. | 5                                                   |
| 2. Basic barium sulfonate blended to 0.96% barium level plus the composition of 1 above.               | 1                                                   |
| 3. Compound 1 (2% active ingredient) plus the composition of 1 above.                                  | 10                                                  |
| 4. Calcium salt of Example 1 blended to 0.28% calcium level plus the composition of 1 above.           | 1                                                   |
| 5. Non-metallic condensation product of Example I, 2% active ingredient plus composition of 1 above.   | 250                                                 |

<sup>1</sup> A commercial dispersant.<sup>2</sup> All carbon black suspended.

As shown by the above data, oil blends containing the calcium salts of the condensation product of Example I are at least equivalent to the commercial dispersant and have superior dispersant properties as compared to blends containing a basic barium sulfonate. Also, as further shown, the non-metallic condensation product imparted excellent dispersant properties as evidenced by a complete suspension of all the carbon black.

Additional tests were carried out with the non-metallic condensation products of this invention in combination with a typical pro-oxidant such as basic barium sulfonate. As shown below in Table V the inhibition of oil blends containing a basic detergent and condensation product 58a was extremely good as shown by the difference in percent viscosity rise between tests 3, 4 and 5.

polymerized ethylene imines having a molecular weight of about 30,000 to 40,000 and an alkylene polyamine of the formula:



in which R is a divalent alkylene radical containing about 2 to 6 carbon atoms and n is an integer from 1 to 10, said phenol and formaldehyde being reacted with said alkylene polyamine in a ratio of about 0.5 to 2 moles of each of said phenol and formaldehyde for each nitrogen atom present in said polyamine to inhibit oxidation.

2. The lubricating oil composition of claim 1 in which the inhibitor-detergent agent is the calcium salt of said condensation product.

3. The lubricating oil composition of claim 1 in which the sulfonate is about 0.5 to 10% of the composition and the condensation product is about 0.1 to 5% of the composition.

20 4. The lubricating oil composition of claim 1 in which the sulfonate is about 0.5 to 10% of the composition and the condensation product is an alkaline earth metal salt present in an amount to provide about .01 to 0.5% of alkaline earth metal in the composition.

25 5. The lubricating oil composition of claim 2 in which said sulfonate is basic barium petroleum sulfonate.

6. The lubricating oil composition of claim 5 in which said alkylene polyamine is tetraethylenepentamine.

30 7. The lubricating oil composition of claim 5 in which said alkylene polyamine is diethylenetriamine.

TABLE V

| Composition of Oil Blend <sup>1</sup>                                                       | Catalyst weight change (mg.) | D-974 acid number | Pentane insol. | pH of oxidized oil | Percent vis. rise | Cat., tube and bubbler    |
|---------------------------------------------------------------------------------------------|------------------------------|-------------------|----------------|--------------------|-------------------|---------------------------|
| 1. Solvent-treated Mid-Continent Neutral Oil, 160 SUS at 100° F...                          | -9.4                         | 1.7               | 0.64           | 4.1                | 9.1               | No sludge, no varnish.    |
| 2. Oil of plus 1% of product 58a of Example 1                                               | -9.0                         | 2.77              | 0.176          | 6.2                | 10                | Sludge and varnish.       |
| 3. Oil of plus basic barium sulfonate blended to 0.96% barium                               | -131                         | 31.12             | 11.32          | 2.1                | 660               | Heavy sludge and varnish. |
| 4. Oil of 1 plus 1% of product 58a of Example I and basic barium sulfonate to 0.96% barium. | -8.8                         | 0.19              | 0.018          | 7.8                | -1.7              | Clean.                    |
| 5. Oil of 1 plus 3% of product 58a of Example I and basic barium sulfonate to 0.96% barium. | -26.4                        | 0.81              | 0.021          | 7.2                | 2.4               | Do.                       |

<sup>1</sup> Concentrations of product 58a are based on the percentage of active ingredients.

I claim:

1. A lubricating oil composition consisting essentially of a mineral lubricating oil containing minor detergent amounts of a basic alkaline earth metal petroleum sulfonate and a minor amount of an oil-soluble inhibitor-detergent agent selected from a member of the group consisting of a condensation product and the alkaline earth metal salts thereof obtained by reacting an alkyl-substituted phenol, in which the alkyl group contains from about 4 to 20 carbon atoms, and formaldehyde with an amine material selected from the group consisting of

References Cited in the file of this patent

UNITED STATES PATENTS

|           |                |               |
|-----------|----------------|---------------|
| 2,353,491 | Oberright      | July 11, 1944 |
| 2,375,222 | Griffin et al. | May 8, 1945   |
| 2,414,729 | Fleming et al. | Jan. 21, 1947 |
| 2,459,112 | Oberright      | Jan. 11, 1949 |
| 2,723,907 | Rogers et al.  | Nov. 15, 1955 |
| 2,725,357 | Kluge et al.   | Nov. 29, 1955 |
| 2,725,358 | Kluge et al.   | Nov. 29, 1955 |
| 2,736,701 | Neff           | Feb. 28, 1956 |